

May 20, 1969

T. J. SARGENT

3,444,573

METHOD OF EFFECTING A TEMPORARY SECUREMENT

Filed July 18, 1967



FIG.-2



FIG.-4



FIG.-1



FIG.-3

INVENTOR  
*Thomas J. Sargent*

BY

*Albert Gordon ATTY*

## 1

3,444,573

**METHOD OF EFFECTING A TEMPORARY SECUREMENT**  
 Thomas J. Sargent, Milford, N.H., assignor to Jacob S. Kamborian, West Newton, Mass.  
 Filed July 18, 1967, Ser. No. 654,106  
 Int. Cl. A43d 9/00, 11/00, 21/00  
 U.S. Cl. 12—142 4 Claims

**ABSTRACT OF THE DISCLOSURE**

There is disclosed herein the temporary attachment of a porous insole to the impervious bottom of a last by means of a cement plug that has a surface adhesion with the last bottom that is released with the passage of time and a mechanical interlock with the insole.

This invention is concerned with the temporary securement of the relatively porous surface of a first member and the relatively impervious surface of a second member by means of a plug of cement interposed between the members in such a manner that when the members are parted the plug is detached from the impervious surface and remains adhered to the porous surface.

In the illustrative embodiment of the invention, the first member takes the form of a relatively porous insole and the second member takes the form of a last having a relatively impervious surface on its bottom. The temporary securement is effected so that shoe manufacturing operations may be performed on the insole-last assembly, after which the insole is separated from the last.

In the drawings:

FIGURE 1 is a plan view of the insole and last prior to securement;

FIGURE 2 is a side elevation showing the pressing of the insole to the last bottom to effect securement;

FIGURE 3 is a cross-section to an enlarged scale of the insole secured to the last bottom by a plug of cement; and

FIGURE 4 is a view of the last-insole assembly with an upper lasted thereto.

The method of this invention is disclosed as being performed by the machine shown in pending application Ser. No. 610,097 filed Jan. 18, 1967. The machine is used to temporarily attach an insole 10 to the bottom of a last 12 by means of plugs of cement 14, 16 and 18. The plug 14 is applied to the last bottom and the plugs 16 and 18 are applied to the insole. The insole 10 is then pressed against the bottom of the last 12, while the last is supported bottom-up, by pressing members 20 and 22 to thereby attach the insole to the last bottom. Conventional shoe manufacturing operations are then performed on the assembled last and insole such as lasting an upper thereto, bottom roughing, outsole attaching, etc. After this, the finished shoe is removed from the last.

The cement utilized is of the delayed tack type and is applied in molten condition to the last bottom and insole. The insole is made of a relatively porous fibrous material such as paperboard or leatherboard and the last bottom is made of a relatively hard impervious material such as wood, plastic or steel.

The delayed tack cement, which is thermoplastic, is composed of an intimate mixture of a resin and a plasticizer. After application to the insole and the last bottom, the cement cools rapidly to room temperature. However, the cement remains in a tacky and fluent condition for a period of time after application to the insole and the last bottom, after which the plasticizer crystallizes and the cement loses its tackiness and fluentness.

## 2

Referring to FIGURE 3, pursuant to the pressing of the insole 10 against the bottom of the last 12 by the pressing members 20 and 22, the cement plugs 14, 16, 18 adhere to the impervious last bottom by surface adhesion without penetrating the last to any substantial extent. Due to the porous nature of the insole, the pressure created by the pressing members 20 and 22 cause the fluent cement plugs 14, 16, 18 to penetrate the interstices of the insole to some extent to thereby adhere to the insole by a mechanical interlock.

The pressing members 20, 22 are released from the insole after enough time has elapsed for the cement plugs to effect an adherence of the insole to the last bottom. After this the shoe manufacturing operations referred to above are performed on the last-insole assembly and the shoe is removed from the last in the conventional manner. Before the plasticizer has crystallized sufficiently to terminate the surface adhesion between the cement plugs and the last bottom, the insole has been anchored to the last by the lasting operation which causes the stretching of the margin 24 of an upper 26, that is mounted on the last, about the last 12 and the attachment of the upper margin, as by cement, to the insole 10 (see FIG. 4). The shoe is removed from the last after sufficient time has elapsed for the plasticizer to crystallize sufficiently so as to terminate the surface adhesion between the cement plugs and the last bottom.

From the foregoing it can be seen that the insole is attached to the last by a permanent mechanical interlock between the cement plugs and the insole and a temporary surface adhesion between the cement plugs and the last bottom. The surface adhesion is retained until after the insole has been anchored to the last bottom by means other than the cement plugs. When the shoe is removed from the last, the cement plugs remain adhered to the insole due to the mechanical interlock and separates from the last bottom due to the termination of the surface adhesion. With this arrangement the last bottom is free of cement so that the last can be used again without scraping any cement particles from its bottom. The plugs of cement adhered to the insole are so thin that they do not create any discomfort to the wearer of the finished shoe.

There are many commercially available delayed tack cements that are suitable for use in the above described method. Each of those used in the illustrative embodiment of the invention comprises a solid, crystalline plasticizer that has been mixed with a resin after the resin has been heated from its normally solid condition into a molten condition to thereby form a molten resin-plasticizer combination. After mixture, the cement is allowed to cool to a solid condition and is stored until it is to be applied to the insole and last bottom at which time it is reheated to a molten condition.

The following are among the cements that can be used. The indicated percentages are by weight. Versamid 940 and Versalon 1160 are supplied by General Mills Chemical Division, Kanakee, Ill., Elvax 40 is supplied by E. I. du Pont de Nemours and Company of Wilmington, Del., Santicizer 9 is supplied by Monsanto Chemical Company of St. Louis, Mo., and Pentaerythritol Tetrabenzoate is supplied by Velsicol Chemical Corporation of Chattanooga, Tenn.

| Cements | Resin                    | Plasticizer                         |
|---------|--------------------------|-------------------------------------|
| 1.....  | 70-80% Versamid 940..... | 20-30% Santicizer 9.                |
| 2.....  | 78% Versalon 1160.....   | 22% Santicizer 9.                   |
| 3.....  | 40% Elvax 40.....        | 60% Pentaerythritol Tetra-benzoate. |

I claim:

1. A method of effecting a temporary securement be-

tween a relatively porous surface of a first member and a relatively impervious surface of a second member comprising: applying at least one plug of cement to at least one of said surfaces, the cement being so constituted as to be initially tacky and to lose its tackiness after the lapse of a time period; pressing the surfaces against each other within said time period so as to cause the cement plug to penetrate said porous surface and adhere thereto by a mechanical interlock and to cause the cement plug to adhere to said impervious surface by a surface adhesion so that an operation may be performed on at least one of said members; and removing the first member from the second member after the lapse of said time period whereby the plug is separated from said impervious surface due to the termination of the surface adhesion and remains adhered to said porous surface due to the mechanical interlock.

2. The method as defined in claim 1 further comprising: effecting an operation on at least one of said members within said time period which causes the members to be anchored to each other by means other than the cement plug.

3. A method of effecting a temporary securement between a relatively porous surface of an insole and a relatively impervious surface of the bottom of a last comprising: applying at least one plugs of cement to at least one of said surfaces, the cement being so constituted as

5 to be initially tacky and to lose its tackiness after the lapse of a time period; pressing the surfaces against each other within said time period so as to cause the cement plug to penetrate said porous surface and adhered thereto by a mechanical interlock and to cause the cement plug to adhere to said impervious surface by a surface adhesion; effecting shoe making operations on the last-insole assembly including an operation, effected within said time period, which causes the insole to be anchored to the last bottom by means other than the cement plug; and removing the insole from the last after the lapse of said time period whereby the plug is separated from the impervious surface of the last bottom due to the termination of the surface adhesion and remains adhered to the porous surface of the insole due to the mechanical interlock.

10 15 20 25 4. The method as defined in claim 3 wherein the said operation effected within said time period consists of the attachment to the insole of the margin of an upper that is mounted on the last.

#### References Cited

#### UNITED STATES PATENTS

|           |        |                |       |        |
|-----------|--------|----------------|-------|--------|
| 2,701,887 | 2/1955 | Nolan          | ----- | 12—142 |
| 2,893,026 | 7/1959 | Sillars et al. | ----- | 12—142 |
| 2,984,847 | 5/1961 | Maeser         | ----- | 12—1   |

PATRICK D. LAWSON, Primary Examiner.